

Sept. 1, 1925.

**1,552,251**

E. C. WASHBURN

## METHOD AND APPARATUS FOR MAKING STEEL INGOTS

Filed May 13, 1922

Fig. 2.



Fig. 3.



Fig. 1.



Fig. 5.



Fig. 6.



Fig. 4.

INVENTOR.  
EDWIN C. WASHBURN.  
BY HIS ATTORNEY.

EDWIN C. WILSON,  
BY HIS ATTORNEY.  
24-  
James F. Williams

## UNITED STATES PATENT OFFICE.

EDWIN C. WASHBURN, OF ENGLEWOOD, NEW JERSEY.

## METHOD AND APPARATUS FOR MAKING STEEL INGOTS.

Application filed May 13, 1922. Serial No. 560,741.

*To all whom it may concern:*

Be it known that I, EDWIN C. WASHBURN, a citizen of the United States, residing at Englewood, in the county of Bergen and

5 State of New Jersey, have invented certain new and useful Improvements in Methods and Apparatus for Making Steel Ingots; and I do hereby declare the following to be a full, clear, and exact description of the 10 invention, such as will enable others skilled in the art to which is appertains to make and use the same.

This invention relates to a method and apparatus for producing iron or steel ingots.

15 It is well known to those skilled in the art that it is now the common practice to cast such ingots in elongated vertical molds. This results in a collection or segregation of impurities in the metal at the upper portion 20 of the ingot and also in what is known as "piping." This latter comprises a formation of a tapering cavity extending downward into the ingot from the top surface substantially at the vertical axis thereof and

25 there is always a collection of impurities adjacent to and extending downward from this "pipe." This necessitates the cutting off of the end of the ingot and the discarding of the same before the ingot is rolled into the desired shapes. In spite of the fact that such a large portion of the ingot is cut away and discarded, the segregation of the impurities and the extension of the "piping" often remains in the part of the ingot used and is 30 rolled out or striated to a narrow dimension during the rolling process, thus forming a faulty section in the material which is often not discovered until the metal fails in use.

It is an object of this invention, therefore, 40 to so cast and produce an ingot that this objectionable piping and segregation of impurities is avoided.

It is a further object of the invention to cast the ingot in an elongated mold which is 45 disposed on its side during the casting operation and which has a gate at the top extending longitudinally thereof so that a projection of metal is formed extending into the gate. The impurities segregate in this 50 projection and the projection is removed after the ingot has solidified to a certain extent.

It is a further object of the invention to

provide an apparatus for casting the ingot comprising an elongated mold having means 55 for supporting the same on its side, said mold having an opening at its top portion extending longitudinally thereof, above which projects a trough forming a pouring gate. 60

It is a further object of the invention to provide such a trough of rectangular cross section having one of its diagonals extending substantially vertical and also to have such a mold formed of sections divided 65 about a vertical central plane of the mold.

These and other objects and advantages of the invention will more fully appear from the following description made in connection with the accompanying drawings which illustrate one form of the apparatus for carrying out the method disclosed herein and in which like reference characters refer to the same parts throughout the different views, and in which, 70

75 Fig. 1 is a view in side elevation of the apparatus, a small portion thereof being shown in section;

Fig. 2 is a view in end elevation of the apparatus; 80

Fig. 3 is a view in vertical section taken on the line 3—3 of Fig. 1, as indicated by the arrows;

Fig. 4 is a partial view in plan of the apparatus; 85

Fig. 5 is a view of another part of the apparatus used in carrying out the method;

Fig. 6 is a view in vertical section taken on the line 6—6 of Fig. 5, as indicated by the arrows; and 90

Fig. 7 is a fragmentary view showing a modified form of the apparatus shown in Figs. 5 and 6.

Referring to the drawings, a mold is shown comprising a rectangular box of elongated shape formed of sections 1 and 2 divided along the central vertical plane of the mold, which mold is disposed with one of its diagonals extending substantially vertically. The mold is closed, save for an opening extending longitudinally along its top, above which opening a trough 3 of flaring formation extends, which trough forms a pouring gate. The sections 1 and 2 are each provided with a groove 4 extending longitudinally along the lower contacting 100

95

100

105

edges, which grooves co-operate to form a channel adapted to receive a sealing substance in the bottom of the mold. The sections 1 and 2 are also each provided with a 5 transverse groove 5 disposed in a projection 6 at the ends thereof, which grooves are adapted to receive a sealing member, such as a common brick which will thus extend across the trough 3 and close the ends thereof. The sections 1 and 2 are further provided at their ends with projecting trunnions or pintles 7 adapted to be engaged by grappling hooks 8 extending from members 9 secured transversely of a longitudinally 10 extending member 10, which latter member carries an eye bolt 11 adapted to be engaged by the hook of a crane. Sections 1 and 2 also have at their ends a lug 12 and receiving channels 13, respectively, adapted 15 to move into engagement and guide the sections 1 and 2 into proper alignment when the said sections are brought together. The sections are also provided at their ends with a locking pin 14 and a locking dog 15, 20 respectively. Said dog having a hook at one end adapted to engage over the pin 14 to hold the sections in assembled position and having a projection 16 at its other end adapted to be pressed upon or struck to 25 disengage the said hook from the pin 14. The apparatus also includes a supporting member for the mold sections 1 and 2 which member comprises spaced transversely extending channel members 17 and spaced vertically inclined diverging channel members 18, the channel members 17 and 18 being 30 connected by vertical plates 19 and 20 and by longitudinally extending plates 21 having their ends bent around and riveted to 35 the plates 19, the plates 19 and 20 being riveted to the channel members 17 and 18. The supporting member thus has the members 18 extending so as to contact and support the lower sides of the mold sections 1 40 and 2 when the mold is in position in the pouring operation.

When the ingot is to be poured the mold is brought into closed position shown in 45 Figs. 1 to 3 and the support therefor will be disposed in convenient relation to the furnace. A piece of common mud or other sealing material will be placed between or in the grooves 4 and a common brick or other frangible member will be placed in the 50 grooves 5. The metal will then be poured in the gate trough 3 and will fill the mold. The impurities tend to segregate at the top 55 of the casting and the same will have easy access to the gate trough 3 and ample opportunity to rise thereto. Such impurities therefore will collect at the top corner of the ingot and in the gate trough 3. It will be noted that the depth of the ingot from the gate being comparatively small, the 60 impurities will have practically no obstruction 65

in rising to the surface of the ingot. The upwardly converging top sides of the mold will not interfere seriously with this movement. The metal will be poured so as to practically fill the gate 3 and there will thus 70 be ample opportunity for the segregation above mentioned.

The metal will be allowed to solidify in the mold and after the same has hardened, but before the ingot is cold, the mold will 75 be lifted from the supporting member and moved to a machine comprising a cutter such as shown in Figs. 5 to 7, which cutter will have blades 22 thereon and will be revolved about its axis 23. The mold will be 80 suitably supported with its top uppermost so that the gate portion will be progressed directly under the cutter blades 22. This cutter will act substantially the same as a milling cutter and will cut or remove a portion of the metal at the top corner of the mold and that portion projecting into the gate 3. If desired, the cutter may be formed with a central notch 24 in the blades, as 85 shown in Fig. 7, so that a corner will be 90 formed on the top edge of the ingot. The metal projecting into the gate trough 3 and at the top edge of the mold will thus be removed and substantially all of the segregated impurities which tend to cause the 95 objectionable "piping" in the ingot will be removed therefrom. The ingot thus produced will be of uniform constituency and formation throughout and when rolled into 100 shapes for use the metal will have a uniform condition of purity.

After the ingot has had the top thereof removed, the mold can be again engaged by the crane and carried to the desired discharging point. It will only be necessary 105 to strike the projection 16 of the dog 15 to release the sections when the same will swing apart owing to converging hook supports 8. The ingot will thus be dropped out of the lower sides of the sections and 110 can be placed as desired. The sections 1 and 2 will be carried back to the supporting device comprising the channel members 18 and as the sections are lowered into the support they will be guided into proper assembled relation by the members 18 and 115 further by the engaging lugs 12 and 13 on the ends of the sections.

From the above description it is seen that 120 applicant has provided a novel and efficient method and apparatus for producing an ingot. The method has been used in actual practice and the ingot produced has given most successful results. The segregated impurities are substantially eliminated and 125 the objectionable "piping" of the ingot avoided. It is thus not necessary to cut away a large section of the ingot containing much good metal in order to eliminate a section of "piping." The saving of metal 130

and labor by the use of the present method and apparatus will be very large and the improved ingot can at the same time be made with great ease and rapidity.

5 It will, of course, be understood that various changes may be made in the form, details and arrangement of the apparatus and in the steps of the method, without departing from the scope of applicant's invention, which, generally stated, consists in the matter shown and described and set forth in the appended claims.

What is claimed is:

1. The process of producing a steel ingot 15 of rectangular cross section, consisting in casting the same in substantially horizontal position with one corner thereof upward.

2. The process of producing a metal ingot of rectangular cross section consisting in 20 casting the same in substantially horizontal position with one corner upward and with a gate member extending longitudinally at the top thereof forming a projection, permitting the ingot to solidify and then removing said projection.

3. The method of producing a metal ingot which consists in casting the same of elongated shape of uniform cross section 30 with its longitudinal side upward and from a gate extending longitudinally of its top side whereby a projection is formed along its top side, allowing the ingot to solidify and before the same has cooled, removing the projection at its top side.

35 4. An apparatus for producing a metal ingot comprising a mold consisting of an elongated divided rectangular box having one corner disposed upwardly and a gate trough extending along and projecting above an opening formed at the top of said box.

5. An apparatus for producing a metal ingot comprising an elongated rectangular mold of uniform cross section, said mold being disposed with one corner upward and divided into sections along a central vertical plane, said mold being closed save for an opening extending longitudinally at its top, and a gate trough projecting above said opening at said corner and extending longitudinally of the mold.

6. The structure set forth in claim 5, said sections having co-operating grooves along the lower meeting edges adapted to receive a sealing substance.

55 7. The structure set forth in claim 5, said trough having transverse grooves adjacent the ends thereof adapted to receive a sealing member for closing the ends of said trough.

60 8. An apparatus for molding a steel ingot, comprising, an elongated mold of rectangular cross section disposed with one diagonal thereof extending substantially vertical, said mold being divided into sections along a central vertical plane, a sup-

port for said mold having upwardly diverging diagonal members adapted to contact with and support the lower surface of said sections and to hold the same in assembled relation.

70 9. The structure set forth in claim 5, said sections having projections at their ends disposed adjacent their outer sides for engagement by a lifting device, whereby said sections will swing apart when lifted.

75 10. The method of producing a metal ingot of rectangular cross section consisting in casting the same with one corner upward and pouring the same throughout the longitudinal extent thereof to form a projecting portion along the top thereof, permitting the ingot to solidify, and then removing said projection before the ingot is cooled with a tool having a recess therein, the sides of which are at right angles to each other 85 whereby a true corner is left on the upper side of the ingot.

80 11. A mold arranged for longitudinal pouring disposed with one corner upwardly and having a gate or feeder portion extending longitudinally thereof at said corner and throughout substantially the entire length of said mold.

90 12. A mold arranged for longitudinal pouring disposed with one corner upwardly and having a riser head portion and an open contracted portion serving as a communication between the mold and said riser portion said portions extending upwardly from said corner.

95 13. A mold comprising relatively movable sections, trunnions thereon, at each side of the longitudinal center line of said sections, links connected to these trunnions, a bar connected to said links and adapted to be raised to swing said sections apart.

100 14. A mold comprising relatively movable sections each having inclined outer sides, and a supporting frame therefor having inclined inner sides adapted to receive said sections and move said sections into alinement when the same are lowered thereinto.

110 15. A mold for a steel ingot comprising, a mold of rectangular cross section disposed with one corner upward and a pouring gate at said corner extending along the entire length of said mold.

115 16. A mold comprising vertically divided sections adapted to seat by gravity in a receiving frame, alined supporting means at the ends and adjacent the outer sides of said sections whereby said sections will swing apart when lifted by said means.

120 17. A mold of rectangular cross section disposed with one corner upwardly, and means disposed at said corner and extending thereabove throughout the length of said mold for pouring metal into said mold.

130 18. A mold comprising separable sections, each section having a recess therein extend-

ing from its inner side, said recess in the respective sections being alined and adapted to receive a sealing member.

19. A mold comprising a plurality of sections, means secured to each section and extending upwardly and outwardly therefrom, a member to which the upper ends of said means are connected whereby when said member is lifted the sections will swing 10 apart.

20. An apparatus for producing a metal ingot comprising an elongated rectangular mold of uniform cross section, said mold being divided into sections along a central vertical plane, said mold being closed save for an opening extending longitudinally at its top and a gate trough projecting above said opening and extending longitudinally of said mold, said trough having transverse

grooves adjacent the ends thereof adapted 20 to receive a sealing member for closing the ends of said trough.

21. An apparatus for molding a steel ingot comprising an elongated mold of substantially uniform cross section, said mold being divided into sections along a central vertical plane, a support for said mold having means for contacting and supporting the lower sides of said sections and tending to hold the same in assembled position. 25

22. The structure set forth in claim 21, said sections having projections at their ends disposed adjacent their outer sides for engagement by a lifting device whereby said sections will swing apart when lifted. 30 35

In testimony whereof I affix my signature.

EDWIN C. WASHBURN.